

## UNITED STATES PATENT OFFICE

EUPHIME V. BERESLAVSKY, OF NEW YORK, N. Y.

## MOTOR FUEL

No Drawing.

Application filed June 18, 1931. Serial No. 545,372.

This invention relates to motor fuels and more particularly to a fuel which will effectively suppress knock in an internal combustion motor.

5 The fuel of the present invention is formed by mixing with the ordinary low compression gasolines on the market a cymene compound which will effectively adapt the fuel for combustion in high compression engines without knocking. This fuel acts to prevent knocking, to maintain the engine cooler during its continued operation and to thereby produce more power by giving the engine more ideal working conditions.

10 The cymenes, particularly ortho, para, meta cymenes and the amino compounds of cymenes when added in small quantities to gasolines or low boiling point hydrocarbons act effectively to produce a gasoline motor fuel which will suppress knock. Para cymene is obtained from wood digestion, particularly the digestion of spruce pulp, and is commonly known as "spruce turpentine". Para cymene also is obtained in comparatively large quantities from high flash naphtha from coke oven oil. That fraction in coke oil boiling between 165° and 190° C. contains approximately 20-35% of tetra methyl benzenes and 20-35% of cymenes. Tetra methyl benzenes are composed largely of durene and iso durene. Para cymene and meta-cymene constitute approximately 20 to 35% of the fraction, and have the formula  $C_{10}H_{14}$ :



Para Cymene



Meta Cymene

25 By nitrating the para cymene and then reducing nitro cymene it is possible to obtain two amino cymenes, namely 2-amino-p-cymene called cymidine or carvacryl amine and 3-amino-p-cymene or thymyl amine. Cymidine is ortho amino para cymene having the following formula:



Cymidine is a liquid having a boiling point of 240° to 242° C. and a melting point less than -16° C. Thymyl amine is meta amino para cymene having the following formula:



Thymyl amine is normally a liquid with a boiling point of 230° C. and a melting point below -15° C.

40 By the nitration and reduction of meta-cymene two amino compounds of cymene may be formed—5 amino-m-cymene and 6-amino-m-cymene—which are normally liquids and have the following formulæ:



50 All of the amino cymene compounds above referred to are directly soluble in the normal gasolines that are found on the market and act as knock suppressors.

55 As the example of knock suppression it has been found that a solution of 20% of cymene and 80% Standard A gasoline in the standard knock testing engine will give the same knock effect as the mixture of 31% pure benzol and 69% Standard A gasoline. The anti-knock value of one per cent by volume of ortho amino para cymene in reference fuel B having 67.6 octane number when tested in standard knock testing engine having a compression pressure 140 lbs./sq. in. with spark advance 15°, was equivalent to 0.4 of a cubic centimeter of tetra ethyl lead, and 4% of ortho amino para cymene in standard fuel B gave the equivalent anti-knock effect in the standard knock engine as 1.6 cubic centimeters of tetra ethyl lead.

60 It has been noted, furthermore, that all of the amino compounds of cymene referred to have the amino group ( $NH_2$ ) attached directly to the carbon nucleus of the aromatic hydrocarbon. Furthermore, the amino compounds of cymene which have been found to be effective knock suppressors have an  $NH_2$  group connected directly to the carbon of the aromatic nucleus and do not have any

other elements connected with the aromatic nucleus except carbon and hydrogen. The compounds which have a molecular structure such as outlined above are entirely consumed in the proper combustion of the motor fuel in the engine and do not produce poisonous compounds which are injurious to health.

Having thus described the above invention, what is claimed as new is:

- 10 1. An anti-knock motor fuel comprising a mixture of low boiling point hydrocarbons and a relatively small proportion of an amino compound of cymene wherein the amino group is attached directly to the carbon of the benzene nucleus.
- 15 2. An anti-knock motor fuel comprising a mixture of low boiling point hydrocarbons

and a relatively small proportion of an amino compound of cymene.

3. An anti-knock motor fuel comprising a mixture of low boiling point hydrocarbons and less than 10 per cent of an amino compound of cymene.

4. An anti-knock motor fuel comprising low boiling point hydrocarbons and a relatively small proportion of an ortho amino para cymene.

5. An anti-knock motor fuel comprising a mixture of low boiling point hydrocarbons and a relatively small proportion of a meta amino para cymene.

In testimony whereof I affix my signature.

EUPHIME V. BERESLAVSKY.

20

85

25

90

30

95

35

100

40

105

45

110

50

115

55

120

60

125

65

130